

[54] NITRASOL PROPELLANT

[75] Inventors: **Joan Reinhart; Warren E. Stump; Julian S. Davidson, all of China Lake, Calif.**[73] Assignee: **The United States of America as represented by the Secretary of the Navy, Washington, D.C.**[22] Filed: **Sept. 16, 1958**[21] Appl. No.: **761,448**[52] U.S. Cl..... **149/18, 149/19, 149/20, 149/76, 149/89, 149/92, 149/96**[51] Int. Cl..... **C06d 5/06**[58] Field of Search..... **52/50, 13, 13.1, 52/5.1; 149/18, 19, 20, 76, 89, 92, 96**

## [56] References Cited

## UNITED STATES PATENTS

2,417,090 3/1947 Silk et al..... 264/3

## FOREIGN PATENTS OR APPLICATIONS

485,662 8/1952 Canada

485,661 8/1952 Canada

## OTHER PUBLICATIONS

Military Explosives, Dept. of the Army Technical Manual, TM-9-1910 Dept. of the Air Force Tech. Order to 11A-1-34 Apr. 14, 1955, p. 247.  
Warren, "Rocket Propellants," Remhold Publ. Corp., N.Y. 1958, p. 37.

Primary Examiner—Benjamin R. Padgett  
Attorney—W. O. Quesenberry and P. H. Firsht

## EXEMPLARY CLAIM

1. A propellant composition consisting essentially of from about 25 to 100 percent binder and up to 75 percent solid loading, said binder comprising from about 10 to 50 percent of plastisol nitrocellulose and from about 15 to 85 percent plasticizer material of the formula  $(O_2 NOCH_2)_3 C-R$  wherein R is a member of the class consisting of hydrogen,  $NO_2$ , lower alkyl and a lower alkyl carbinol radical, said solid loading consisting of up to 60 percent of a metal and from about 20 to 100 percent of a material from the class consisting of perchlorate oxidizing agents, cyclotetramethylene tetranitramine, trinitroethylorthocarbonate and mixtures thereof; said plastisol nitrocellulose being made by placing 90 grams of nitrocellulose (12.6 percent N), 1.2 grams of ethyl centralite and 1.4 liters of nitromethane in a flask and stirring vigorously until dissolution occurs, stirring slowly for an additional 10 minutes to insure homogeneity, adding to the resulting lacquer 19.2 grams of a petroleum sulfonate emulsifying agent for nitrocellulose in about 900 ml of water and circulating through a colloid mill for about 10 minutes, draining the resulting emulsion from the mill into about 30 liters of water and stirring about 15 minutes until a nitrocellulose precipitate is formed which is filtered from the liquid, washed in hexane, dried for about 16 hours and sifted through a 200 mesh screen.

5 Claims, No Drawings

## NITRASOL PROPELLANT

The invention herein described may be manufactured and used by or for the Government of the United States of America for governmental purposes without the payment of any royalties thereon or therefor.

This invention relates to rocket propellants; more specifically it relates to improved propellant binders.

In the past, many propellants have been developed, but the best of these has a specific impulse of only about 240 lb-sec/lb. A rocket propelled with such a propellant of course has performance limitations due to the energy limitations of the propellant.

Propellant grains often cannot stand the stresses of great temperature changes, or ignition without cracking. As is well known, a cracked grain when fired usually results in a ruptured motor tube.

Propellants utilizing a resinous binder usually have a pot life of only a few hours; once the components are mixed, rapid casting is necessary so that the propellant will not cure before it is shaped.

The propellants of today which are capable of specific impulses of 240 lb-sec/lb are of the composite type which contain an oxidizer and light metal incorporated in a polymeric binder. After prolonged storage, the oxidizer tends to migrate away from the surface of the grain, making the grain difficult to ignite.

It is therefore an object of this invention to provide rocket propellants which have higher specific impulses than previous propellants.

Another object is to provide propellants which will not crack under the stresses of ignition or stresses caused by expansion and contraction due to extreme changes in temperature.

Still another object is to provide propellants having a relatively long pot life, being measured in weeks instead of hours.

A final object is to provide a grain which will ignite reliably even after long periods of storage.

The above objects are accomplished by an elastomeric high energy binder which incorporates a solid oxidizer with or without a light metal fuel and which may be cast into a motor tube and cured in situ. The binder alone or in combination with an oxidizer is a fairly good propellant but when loaded with the oxidizer and metals aforementioned, gives especially high energy formulations. The solids loading runs as high as 75 percent by weight.

The binder consists of a mixture of from about 15 to 85 percent high energy plasticizer, zero to 20 percent inert plasticizer, and about 10 to 50 percent plastisol nitrocellulose. The high energy plasticizer is one selected from the group consisting of primary and secondary nitrate esters, both liquid and solid. Preferred nitrate esters are pentaerythritol trinitrate and trimethylolethane trinitrate.

The inert plasticizer is conventional and may or may not be added to modify ballistic and physical properties. Dibutyl phthalate is commonly employed as such a plasticizer.

Plastisol nitrocellulose is made in batches by placing 90 gms of dry nitrocellulose (12.6 percent N), 1.2 gms ethyl centralite, and 1.4 liters of nitromethane in a flask and stirring vigorously until apparent dissolution occurs, then stirring slowly for 10 minutes more to insure homogeneity in the resulting lacquer. About 19.2 gms of a suitable petroleum sulfonate emulsifying agent, for example Petromix No. 9, in about 900 ml of water is

added to the lacquer and the mixture circulated and recirculated through a colloid mill wherein the liquid has to pass between a stator and a rotor which have only a small clearance while the rotor rotates at about 10,000 rpm.

After 10 minutes, the emulsion is drained from the colloid mill into about 30 liters of stirred water and stirred for about 15 minutes whereupon a precipitate of nitrocellulose forms. Then the precipitate is filtered out of the liquid, washed in hexane and dried for about 16 hours. Then the nitrocellulose is sifted through a 200 mesh screen.

The above procedure yields dense, spherical nitrocellulose particles of 1 - 30 $\mu$  median diameter. This form of nitrocellulose is not substantially attacked by the plasticizers until cure at elevated temperature is initiated.

Small amounts of conventional stabilizers are added in accordance with good practice. Ethyl centralite and N-methyl-p-nitroaniline are widely used to stabilize nitrocellulose.

The solids which are incorporated in the binder to make the improved propellant are normally ammonium perchlorate and a metal such as aluminum, magnesium, boron, zirconium and titanium. Other perchlorate and nitrate oxidizers could be used. Particle size is not critical from the standpoint of operability but does affect the burning rate. The smaller the particle size, the more rapid the burning rate, generally.

The proportion of aluminum or other light metal may run as high as 60 percent of the weight of the propellant.

The propellant is made by placing the powdered plastisol nitrocellulose in a sigma blade mixer and pouring in about 45 percent of the liquid plasticizer (s). The mixture is agitated for about 15 minutes. Then the remainder of the plasticizer (s) is added and the mixture agitated for about 30 minutes under vacuum to remove entrapped air.

The powdered metal is added, if metal is to be used, and stirred into the mixture until it is thoroughly wetted; the solid oxidizer is added and the mixture agitated again for about 30 minutes under vacuum. During the last 15 minutes, warm water at 110° F. is run through the jacket surrounding the mixer in order to bring the temperature of the mixture up to 110° F. Then the mixing is discontinued and the mixture simply poured into a rocket motor tube, in the absence of pressure or vacuum, and the tube placed in an oven and maintained at 185° F. for 1 to 2 hours. At the end of the period, the propellant is cured and ready for firing. A pentaerythritol trinitrate containing binder can be stored for several days at room temperature and a trimethylolethane trinitrate containing binder even longer without curing.

In Table I which follows there is given a comparison of two different high energy binders.

TABLE I

|                                                        | Binder<br>1 | Type<br>2 |
|--------------------------------------------------------|-------------|-----------|
| 60 Composition and Properties                          |             |           |
| Nitrocellulose (12.6% N), %                            | 28.5        | 28.5      |
| Trimethylolethane trinitrate, (TMETN) %                | 70          | —         |
| Pentaerythritol trinitrate, (PETRIN) %                 | —           | 70        |
| Ethyl centralite, %                                    | 1.5         | 1.5       |
| 65 Heat of Explosion, cal/g                            | 996         | 1043      |
| Viscosity, 77°F., Poises                               | 5           | 30        |
| Tensile strength <sup>a</sup> at rupture, psi<br>77°F. | 192         | 242       |
| 0°F.                                                   | 1340        | 1768      |

|                                    |      |      |  |  |
|------------------------------------|------|------|--|--|
| Elongation <sup>a</sup> , %        |      |      |  |  |
| 77°F.                              | 107  | 128  |  |  |
| 0°F.                               | 80   | 62   |  |  |
| Closed-bomb specific impulse, sec. | 222  | 216  |  |  |
| Taliani, mm Hg/minute              | 0.72 | 0.44 |  |  |

<sup>a</sup>obtained from duplicate specimens cut from propellant sheets 1/4 inch thick.

Of particular interest is the low viscosity of binder 1 in the uncured state which affords higher solids loading and greater flexibility in propellant formulation because of a wider range of possible compositions with good castability.

The energies of the two binders do not vary much but, the TMETN containing binder seems to be more elastomeric at temperatures in the neighborhood of 0° F., and both are more elastomeric than double-base propellants at any temperature; TMETN has the additional advantage over PETRIN that it allows the nitrocellulose to be cross-linked with a diisocyanate to produce a stronger grain.

Table II which follows shows the effect of loading a particular binder with varying amounts of oxidizer.

TABLE II

| Composition and properties                       | Example |       |       |       |      |
|--------------------------------------------------|---------|-------|-------|-------|------|
|                                                  | 1       | 2     | 3     | 4     | 5    |
| Ammonium perchlorate, 200μ, percent              | 20      | 30    | 40    | 50    | 60   |
| Binder, percent                                  | 80      | 70    | 60    | 50    | 40   |
| Heat of explosion, cal./g.                       | 893     | 1,012 | 1,160 | 1,327 |      |
| Burning rate (1,000 p.s.i. and 80° F.), in./sec. | 0.29    | 0.27  | 0.34  | 0.38  | 0.41 |
| Pressure exponent                                | 0.52    | 0.43  | 0.48  | 0.47  | 0.53 |
| Taliani, mm. Hg/minute                           | 1.0     | 0.9   | 0.7   | 0.6   | 0.6  |

<sup>a</sup> Binder composition, weight percent: Nitrocellulose (12.6% N) 38, Petrin 39, dibutyl phthalate 20, adiponitrile 1, ethyl centralite 2.

As is readily apparent, the heat of explosion, burning rate and Taliani stability increase with increased oxidizer loading, while the pressure exponent of burning varies moderately.

Table III below shows the effect of including aluminum along with an oxidizer in a particular binder to form the propellant.

The inclusion of aluminum has increased the heat of explosion considerably over those formulations not containing it, as is to be expected, while other properties do not vary greatly.

TABLE III

| Composition and Properties | Example |      |      |      |
|----------------------------|---------|------|------|------|
|                            | 1       | 2    | 3    | 4    |
| Ammonium perchlorate       | 21.5    | 30   | 23.5 | 27.0 |
| Aluminum, atomized         | 21.5    | 20   | 21.5 | 23.0 |
| Nitrocellulose (12.6% N)   | 16.2    | 17.1 | 19.0 | 14.3 |
| PETRIN                     | 39.9    | 27.0 | 35   | 35   |
| Dibutyl phthalate          | —       | 5    | —    | —    |
| Ethyl centralite           | 0.9     | 0.9  | 1.0  | 0.7  |

5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

aluminum, but the binder composition varies in each case. All the formulations are sufficiently elastomeric to be case bonded to motor tubes. HMX (cyclotetramethylene tetranitramine) and TNEOC (trinitroethyl-orthocarbonate), are high energy additives which may be used, sometimes completely replacing the ammonium perchlorate oxidizer.

Table VI which follows shows the effects of these additives.

TABLE VI

| Composition and properties                      | Example |                 |       |                 |       |
|-------------------------------------------------|---------|-----------------|-------|-----------------|-------|
|                                                 | 1       | 2               | 3     | 4               | 5     |
| Binder type a                                   | G       | G               | G     | H               | H     |
| HMX, 100 avg. percent                           | 37      | 22              | 20    | 30              | 30    |
| TNEOC, percent                                  | 32      |                 |       |                 |       |
| Ammonium perchlorate, percent                   |         |                 | 12    |                 |       |
| Aluminum, atomized, percent                     | 18      | 13              | 16    | 20              | 20    |
| Burning rate, 70° F. and 1,000 p.s.i., in./sec. | 0.35    | 0.15            | 0.22  | 0.34            | 0.3   |
| Pressure exponent                               | 1.0     | 0.9             | 0.6   | 0.7             | 0.8   |
| Heat of explosion, cal./g.                      | 1,057   | 908             | 1,079 | 1,433           | 1,490 |
| Tialian, mm. Hg/minute                          | 1.4     | 0.3             | 0.5   | 0.3             | 0.3   |
| Impact sensitivity, 50% point, cm.              |         | 33 <sup>b</sup> |       | 25 <sup>b</sup> |       |

a See the following table:

|                                      | G  | H    |
|--------------------------------------|----|------|
| Binder formulations, weight percent: |    |      |
| Nitrocellulose (12.6% N)             | 38 | 28.5 |
| Petrin                               | 39 | 70   |
| Dibutyl phthalate                    | 20 |      |
| Adiponitrile                         | 1  |      |
| Ethyl centralite                     | 2  | 1.5  |

b Uncured.

HMX causes a marked decrease in burning rate and produces a higher pressure exponent than that obtained with ammonium perchlorate. TNEOC exhibits fair heat stability and is less sensitive to impact than ammonium perchlorate.

Table VII below presents specific impulses calculated from static firing data. Theoretical calculations for the specific impulses of these propellants range from 240 - 265 lb-sec./lb. The propellant contains 50 percent solids loaded into the binder E of Table IV except in examples 9 and 10 where binder D is used, and the specific impulse is measured as a function of the aluminum content.

TABLE VII

| Example | Aluminum Content<br>WT. % | Isp<br>at 1000<br>psi |
|---------|---------------------------|-----------------------|
| 1       | 25                        | 249                   |
| 2       | 20                        | 227                   |
| 3       | 20                        | 224                   |
| 4       | 15                        | 240                   |
| 5       | 15                        | 243                   |
| 6       | 15                        | 241                   |
| 7       | 10                        | 274                   |
| 8       | 10                        | 235                   |
| 9       | 15                        | 235                   |
| 10      | 15                        | 255                   |

The ballistic and physical properties presented in the foregoing tables were measured by standard techniques well known in the art.

The propellants are acceptable for military purposes as relates to surveillance, electrostatic sensitivity and friction sensitivity.

From the foregoing it is evident that propellants with excellent physical properties have been produced which are sufficiently elastomeric to be case bonded to motor tubes. Excellent ballistic properties are also displayed by the formulations. The binder can be mixed and stored for as long as two weeks at room temperature without curing.

Obviously many modifications and variations of the present invention are possible in the light of the above teachings. It is therefore to be understood that within

the scope of the appended claims the invention may be practiced otherwise than as specifically described.

What is claimed is:

1. A propellant composition consisting essentially of from about 25 to 100 percent binder and up to 75 percent solid loading, said binder comprising from about 10 to 50 percent of plastisol nitrocellulose and from about 15 to 85 percent plasticizer material of the formula  $(O_2 NOCH_2)_3 C - R$  wherein R is a member of the class consisting of hydrogen,  $NO_2$ , lower alkyl and a lower alkyl carbinol radical, said solid loading consisting of up to 60 percent of a metal and from about 20 to 100 percent of a material from the class consisting of perchlorate oxidizing agents, cyclotetramethylene tetranitramine, trinitroethylorthocarbonate and mixtures thereof; said plastisol nitrocellulose being made by placing 90 grams of nitrocellulose (12.6 percent N), 1.2 grams of ethyl centralite and 1.4 liters of nitromethane in a flask and stirring vigorously until dissolution occurs, stirring slowly for an additional 10 minutes to insure homogeneity, adding to the resulting lacquer 19.2 grams of a petroleum sulfonate emulsifying agent for nitrocellulose in about 900 ml of water and circulating through a colloid mill for about 10 minutes, draining the resulting emulsion from the mill into about 30 liters of water and stirring about 15 minutes until a nitrocellulose precipitate is formed which is filtered from the liquid, washed in hexane, dried for about 16 hours and sifted through a 200 mesh screen.
2. A propellant composition consisting essentially of about 10 to 50 percent plastisol nitrocellulose and from about 15 to 85 percent of a plasticizer material of the formula  $(O_2 NOCH_2)_3 C - R$  wherein R is a member of the class consisting of hydrogen,  $NO_2$ , lower alkyl and a lower alkyl carbinol radical, said plastisol nitrocellulose being made by vigorously stirring until dissolution 90 grams of dry nitrocellulose (12.6 percent N), 1.2 grams of ethyl centralite, and 1.4 liters of nitromethane in a flask, and slowly stirring for about 10 additional minutes to insure homogeneity, adding to the resulting lacquer about 19.2 grams of a petroleum sulfonate emulsifying agent for the nitrocellulose, 900 ml of water and circulating the mixture thereof through a colloid mill for about 10 minutes after which the emulsion therefrom is drained from the mill into about 30 liters of water and stirred for about 15 minutes whereupon the nitrocellulose containing precipitate forms which is filtered, washed in hexane, dried for about 16 hours and sifted through a 200 mesh screen.
3. A propellant composition consisting essentially of from about 35 to 55 percent of a binder which comprises from about 10 to 50 percent plastisol nitrocellulose, about 15 to 85 percent of a plasticizer selected from the group consisting of pentaerythritol trinitrate and trimethylethane trinitrate, about 15 to 20 percent aluminum and from about 30 to 35 percent ammonium perchlorate, said plastisol nitrocellulose being made by placing 90 grams of nitrocellulose (12.6 percent N), 1.2 grams of ethyl centralite and 1.4 liters of nitromethane in a flask and stirring vigorously until dissolution occurs, stirring slowly for an additional 10 minutes to insure homogeneity, adding to the resulting lacquer 19.2 grams of a petroleum sulfonate emulsifying agent for nitrocellulose in about 900 ml of water and circulating through a colloid mill for about 10 minutes, draining the resulting emulsion from the mill into about 30 liters of water and stirring about 15 minutes until a nitrocellulose precipitate is formed which is filtered from the liquid, washed in hexane, dried for about 16 hours, and sifted through a 200 mesh screen.
4. The propellant composition of claim 3 in which cyclotetramethylene tetranitramine is substituted for ammonium perchlorate.
5. The propellant composition of claim 3 in which trinitroethylorthocarbonate is substituted for ammonium perchlorate.

\* \* \* \* \*